

# UNITED STATES PATENT OFFICE.

EUGENE A. BYRNES, OF WASHINGTON, DISTRICT OF COLUMBIA, ASSIGNOR TO PITTSBURGH PURE METAL PRODUCTS COMPANY, OF PITTSBURGH, PENNSYLVANIA, A CORPORATION OF PENNSYLVANIA.

## IRON-SILICON INGOT.

1,004,987.

Specification of Letters Patent.

Patented Oct. 3, 1911.

No Drawing.

Application filed January 28, 1911. Serial No. 605,298.

*To all whom it may concern:*

Be it known that I, EUGENE A. BYRNES, a citizen of the United States, residing at Washington, in the District of Columbia, 5 have invented certain new and useful Improvements in Iron-Silicon Ingots, of which the following is a specification.

It is now well recognized that ordinary Bessemer and open-hearth steels rust more 10 readily than wrought or puddled iron, and that the manganese commonly used as a de-oxidizing addition in the production of such steels is apt to segregate and increases the rate of corrosion.

15 The present invention is a cast ingot, for conversion into such commercial shapes and articles as are exposed to atmospheric and oxidizing influences, consisting almost entirely of iron; containing very little carbon,

20 sulfur, phosphorus, manganese, oxygen and nitrogen; and having alloyed therewith a small amount of silicon. The preferred product contains up to 99.7 per cent. of iron; not over 0.15 total per cent. of carbon, sulfur, 25 phosphorus, manganese, oxygen and nitrogen; and 0.15 per cent. or more of silicon. This product is preferably manufactured in the basic open-hearth with basic additions, from a charge of pure pig iron and wrought-

30 iron scrap. The temperature is raised to and maintained at a high point throughout the purification, without unduly increasing the oxidizing character of the flame, until the carbon, sulfur, phosphorus, manganese and

35 silicon have been reduced to a total per cent. of not over 0.15. The combined oxygen is preferably removed by the use of both silicon and titanium, the latter also serving to practically eliminate the nitrogen.

40 The silicon may be added in the form of the 50% ferro-alloy; the titanium as a 30%

ferro-alloy. The ferro-alloys may be added at the end of the purifying stage, or portions of them may be added toward the end of the treatment. The silicon is added in 45 such excess as to leave the desired per cent., say from 0.10 to 0.15 in the finished product. The titanium is preferably added in the minimum amount necessary to eliminate oxygen and nitrogen. In some cases it may 50 be desirable, in order to readily obtain a high temperature and facilitate the final reaction, to tap the metal from the open-hearth furnace into an electric furnace. The slag may then be largely removed in transit, 55 a neutral atmosphere being maintained in the electric furnace.

I claim:—

1. As a new article of manufacture, a cast ingot containing at least 99.5 per cent. of 60 iron; not over 0.15 total per cent. of carbon, sulfur, phosphorus and manganese; and at least 0.10 per cent. of silicon.

2. As a new article of manufacture, a cast ingot containing at least 99.5 per cent. of 65 iron; not over 0.15 total per cent. of carbon, sulfur, phosphorus, manganese, oxygen and nitrogen; and at least 0.10 per cent. of silicon.

3. As a new article of manufacture, a cast 70 ingot containing from 99.5 to 99.7 per cent. of iron; not over 0.15 total per cent. of carbon, sulfur, phosphorus, manganese, oxygen and nitrogen; and at least 0.15 per cent. of silicon. 75

In testimony whereof, I affix my signature in presence of two witnesses.

EUGENE A. BYRNES.

Witnesses:

ROBERT I. HULSIZER,  
JOHN H. SIGGERS.